

## UNITED STATES PATENT OFFICE.

GEORGES HEBERLEIN, OF WATTWIL, SWITZERLAND, ASSIGNOR TO HEBERLEIN PATENT CORPORATION, OF NEW YORK, N. Y., A CORPORATION OF NEW YORK.

## PROCESS FOR PRODUCTION OF PERMANENT EFFECTS IN COTTON FABRICS.

No Drawing. Application filed September 1, 1921. Serial No. 497,740. Renewed November 15, 1922. Serial No. 601,038.

(GRANTED UNDER THE PROVISIONS OF THE ACT OF MARCH 3, 1921, 41 STAT. L., 1313.)

To all whom it may concern:

Be it known that I, GEORGES HEBERLEIN, a citizen of the Swiss Republic, and a resident of Wattwil, Canton of St. Gall, Switzerland, have invented certain new and useful Improvements in Processes for Production of Permanent Effects in Cotton Fabrics (which improvements are described in the following filed applications, i. e., German application Ser. No. 65,355, filed Feb. 13, 1914, patent of addition #292,213, granted May 26, 1916; German application Ser. No. H. 68,470, filed May 19, 1915, Patent #295,816, granted Dec. 18, 1916; French application Ser. No. 83,050, filed Apr. 21, 1916, Patent #481,561, granted Sept. 23, 1916; British application Ser. No. 6,218 of 1916, filed May 1, 1916, Patent #100,483, granted as of May 19, 1915; Belgian application Ser. No. 225,208, filed June 24, 1919, Patent #280,937, granted (not yet issued); Italian application Ser. No. (have none), filed May 4, 1916, Patent #154,095, granted June 5, 1916; Austrian application Ser. No. 25 (have none), filed Apr. 29, 1916, Patent #81,367, granted Sept. 25, 1920), of which the following is a specification.

My invention relates to a process of treating cotton fabric to produce wool-like effects. In my United States Patent No. 1,141,872, granted June 1, 1915, I have described and claimed a process of treating cotton fabric to produce permanent wool-like effects, by first mercerizing the fabric and then treating it with concentrated sulphuric acid of less than 51° Bé. It was described in that patent specification that if cotton fabric which has been mercerized and also preferably bleached, be subjected to the action of sulphuric acid of from 49° to somewhat under 51° Bé. (the best action being obtained between 49½ deg. and 50½ deg. Bé.), the mercerizing lustre disappears, and instead of the transparency obtained with the higher concentration of sulphuric acid, the fabric assumes a fine light crape-like nature, whereby it appears fuller, more wool-like, softer, and is generally improved and it has imparted to it somewhat the character of fine woolen stuff, such for example as fine thin wool muslin.

It was also pointed out in that patent that

the treatment could be utilized in the method described for producing pattern effects. It was pointed out that pattern effects could be produced on plain fabrics by printing on mercerized fabrics with sulphuric acid of say 50° Bé. and washing out after action has taken place; or that a suitable resist such as gum thickening could be impressed on portions of the fabric in such a way as to protect the parts not to be acted upon by the acid, and then the entire fabric dipped into sulphuric acid of the aforesaid concentration, and subsequently washing the fabric.

I have also discovered that the wool-like quality of the fabric mentioned in said Patent No. 1,141,872 is also obtained if the cotton fabric is first treated with the sulphuric acid of from 49° to 51° Bé., then washed, and without stretching, mercerizing the fabric with caustic alkali such as caustic soda. The latter process forms the subject matter of my co-pending application Serial Number 497,738 filed on even date herewith.

The latter process is distinguished from that described in the aforesaid patent, in that the said wool effect is obtained according to the process of the aforesaid patent, regardless of whether the mercerizing is carried out with or without stretching, whereas in said latter process where the mercerizing is carried out after the acid treatment, the proper wool-like effect takes place only when the mercerizing is done without stretching.

I have further discovered that the said wool-like effect is attained if in carrying out the above described processes, the treatment with sulphuric acid is replaced by a treatment with phosphoric acid of 55° to 57° Bé., or with hydrochloric acid of the specific gravity of 1.19 at low temperature (as for example below 0° C.) or with nitric acid of 43° to 46° Bé., or with zinc chloride solution of 66° Bé., at 60° to 70° C. or with Schweizer's solution, with a short reaction period.

In this application for Letters Patent I aim to cover the above described processes wherein hydrochloric acid is utilized in conjunction with the mercerizing process instead of the sulphuric acid. The remainder of the improvements herein described are covered by other of my co-pending applications and patents.

It will be understood by those skilled in the art that when the cotton fibres are treated as herein stated, the fibres are chemically structurally changed by each treatment, and it is a characteristic of fabrics treated according to my process, that the fibres are chemically structurally changed, and that the changed or altered condition of the fibres is permanent, i. e., will withstand repeated laundering so that the goods may be laundered without eliminating or materially altering the characteristics of the fabric above described, and this greatly enhances their value.

Having thus described my invention, what I claim as new and desire to secure by Letters Patent, is:

1. Method of treating cotton fabric to produce a fabric in which the fibres have been chemically structurally altered to give to the fabric a different and pleasing appearance which is permanent, which method comprises subjecting the fabric to two chemical treatments, one a mercerizing treatment, and the other a treatment with hydrochloric acid to differently structurally change the fibres, the fabric being subjected to one of said treatments after the other, and after the acid treatment washing the fabric.

2. Method of treating cotton fabric to produce a fabric in which the fibres have been chemically structurally altered to give to the fabric a different and pleasing appearance which is permanent, which method comprises subjecting the fabric to two chemical treatments, one a treatment with caustic soda which will chemically structurally change the fibres, and the other a

treatment with hydrochloric acid of the specific gravity of 1.19 at low temperature.

3. Method of treating cotton fabric to chemically structurally change the fabric so as to produce a wool-like effect, which method comprises subjecting the fabric to two chemical treatments, one a mercerizing treatment, and the other a treatment with hydrochloric acid at low temperature, and after the acid treatment washing the fabric.

4. Method of treating cotton fabric to chemically structurally change the fabric so as to produce the described wool-like effect, which method comprises subjecting the fabric first to a mercerizing treatment, and thereafter to a treatment with hydrochloric acid at low temperature, and then washing the fabric.

5. Method of treating cotton fabric to chemically structurally change the fabric so as to produce the described wool-like effect, which method comprises subjecting the fabric first to a mercerizing treatment with caustic soda, and thereafter subjecting it to a treatment with hydrochloric acid of specific gravity of 1.19 at low temperature, and then washing the fabric.

6. Method of treating cotton fabric to chemically structurally change the fabric so as to produce a wool-like effect, which method comprises subjecting the fabric to two chemical treatments, one a treatment with caustic alkali, and the other a treatment with hydrochloric acid which, in conjunction with the alkali treatment, will produce the said wool-like effect.

In testimony whereof I have signed my name to this specification.

GEORGES HEBERLEIN.

**Certificate of Correction.**

It is hereby certified that in Letters Patent No. 1,439,520, granted December 19, 1922, upon the application of Georges Heberlein, of Wattwil, Switzerland, for an improvement in "Processes for Production of Permanent Effects in Cotton Fabrics," an error appears in the printed specification requiring correction as follows: Page 1, lines 28 and 29, strike out the words "process of treating cotton fabric to produce wool-like effects" and insert instead *process for production of permanent effects in cotton fabrics*; and that the said Letters Patent should be read with this correction therein that the same may conform to the record of the case in the Patent Office.

Signed and sealed this 3d day of April, A. D., 1923.

[SEAL.]

**KARL FENNING,**  
*Acting Commissioner of Patents.*